

3,679,493

**GLYCOL ETHER-CHROMIUM CORROSION RESISTANT COATINGS FOR METALLIC SURFACES**  
 John Paul Gerhardt Beiswanger, Easton, and Assadullah Nassry, Bethlehem, Pa., assignors to GAF Corporation, New York, N.Y.  
 No Drawing. Filed Mar. 11, 1970, Ser. No. 18,762  
 Int. Cl. C23f 7/26, 11/16

U.S. Cl. 148—6.16

21 Claims

## ABSTRACT OF THE DISCLOSURE

A process and composition for increasing the resistance to corrosion of a metallic surface, which process comprises contacting said metallic surface with a composition obtained by mixing in the presence of water a water soluble chromium compound such as chromium trioxide, ammonium chromate, chromium chromate, and the like, and an oxygenated organic compound having the following formula:



wherein  $\text{R}_1$  is an alkyl group having from 1 to 6 carbon atoms,  $\text{R}_2$  is hydrogen or an alkyl group having from 1 to 6 carbon atoms, and  $\text{R}_3$  is hydrogen or an alkyl group having from 1 to 6 carbon atoms,  $n$  is an integer of from 1 to 4.

## FIELD OF THE INVENTION

The instant invention relates to a composition useful in increasing the corrosion resistance of metallic surfaces and a process for protecting metallic surfaces by the application of such compositions thereto. In particular, the instant invention is directed to the use of a composition comprising a chromium compound and an oxygenated organic compound (I) to increase the corrosion resistance of metallic surfaces.

## PRIOR ART

Heretofore, a number of surface treating processes have been proposed in order to solve a problem in connection with the corrosion resistance or adherence of finish coatings to the metal surface. For example, it is known that the phosphating treatment involving the use of a phosphate solution, such as, iron, zinc, manganese or calcium phosphate, or an electrolytic treatment in a phosphate or chromate solution with an alternating or direct electric current, will afford some measure of corrosion resistance. Although the above processes have attained some measure of corrosion resistance, ease of adaptability for commercial fabrication, poor adherence, and only marginally improved corrosion resistance have rendered the prior art approaches incompletely acceptable. A somewhat thick film resulting from the prior art surface treatment is required in order to effect corrosion resistance and such films provide poor handling characteristics. The poor adherence of such thick finished coatings to the treated substrate compounds the problem even further.

Other processes have been employed to increase the resistance of metallic surfaces to corrosion, which processes include the use of an oxygenated organic compound. It is noted, however, that in each of these attempts, the compositions employed also contained additional ingredients such as polymeric materials, a multiplicity of reducing agents, fillers, and the like. As distinguished therefrom, the composition of the instant invention is a relatively simple one which includes a solution of the

reaction product of a water soluble chromium compound with an oxygenated organic compound as the essential ingredient thereof. While other materials may be added to the instant composition, they are not essential to the effectiveness thereof.

Therefore, it is an object of the instant invention to provide improved corrosion resistant coatings for metallic surfaces.

Another object of the instant invention is to provide for a process of improving the corrosion resistance of metallic surfaces.

## THE INVENTION

These and other objects of the instant invention are achieved by the provision of a corrosion-resistant coating consisting essentially of the reaction product of a water soluble chromium compound with an oxygenated organic compound in the presence of water.

## DETAILED DESCRIPTION

20 The composition of the instant invention is considered particularly useful in protecting ferrous metallic surfaces in general such as iron and steel plate or castings, tin coated and zinc coated (galvanized) iron and steel and other ferrous alloys. Other metallic surfaces which may be protected by the composition and product of this invention include non-ferrous substrates such as zinc surfaces, aluminum surfaces, magnesium surfaces, tin surfaces, and non-ferrous alloy surfaces such as brass, bronze and the like.

25 As previously noted, one of the essential ingredients of the instant composition is a water-soluble chromium compound. The useful chromium compounds include, but are not limited to, chromium trioxide, ammonium chromate, zinc chromate, chromium chromate, chromic acid, potassium dichromate, and mixtures thereof. It is, of course, within the scope of the instant invention to employ other chromium salts similar to the above which are soluble in the reaction medium.

30 The useful oxygenated organic compounds generally have the formula:



35 wherein  $\text{R}_1$  represents an alkyl group having from 1 to 6 carbon atoms,  $\text{R}_2$  and  $\text{R}_3$  represent hydrogen or an alkyl group having from 1 to 6 carbon atoms, and  $n$  is an integer of from 1 to 4. Representative of compounds included in the above general formula are the following:

- 45 Ethylene glycol monomethylether
- Ethylene glycol dimethylether
- Ethylene glycol monoethyl ether
- Ethylene glycol diethyl ether
- 50 Ethylene glycol monobutyl ether
- Ethylene glycol dibutyl ether
- Ethylene glycol monoisobutyl ether
- Ethylene glycol diisobutyl ether
- Ethylene glycol monoamyl ether
- 55 Ethylene glycol diethyl ether
- Ethylene glycol mono-n-hexyl ether
- Ethylene glycol monomethyl ether
- 60 Diethylene glycol dimethyl ether
- Diethylene glycol monoethyl ether
- Diethylene glycol monobutyl ether
- Diethylene glycol dibutyl ether
- Diethylene glycol monoisobutyl ether
- 65 Diethylene glycol diisobutyl ether
- Triethylene glycol monomethyl ether
- 70 Triethylene glycol dimethyl ether
- Triethylene glycol diethyl ether

Triethylene glycol monoethylether  
 Tetraethylene glycol monomethylether  
 Tetraethylene glycol dimethylether  
 Propylene glycol monomethylether  
 Propylene glycol dimethylether  
 Propylene glycolmonoethylether  
 Propylene glycol diethylether  
 Propylene glycol monobutylether  
 Butylene glycol monoethylether  
 Butylene glycol monobutylether  
 The monomethyl ether of mixed ethylene/propylene glycol  
 The monomethyl ether of mixed ethylene/butylene glycol.

In addition to the above two essential ingredients, i.e., the water-soluble chromium compound and the aforesaid oxygenated organic compound, one may also employ in connection with the composition of the instant invention various compatible wetting agents to improve the surface wetting and coating uniformity of said composition. It is noted that the wetting agent employed must be one which is compatible with, and stable in the presence of, the chromium compound employed in the instant invention. Therefore, preferably, one employs as the wetting agent a nonionic or anionic surfactant material although other types of surfactants may also be employed if compatible under the conditions of use. Representative of the surfactants which may be employed are the following:

- (1) Alkylaryl sulfonates such as sodium alkylnaphthalene sulfonate.
- (2) Alkyl sulfates such as sodium lauryl sulfate.
- (3) The sulfonated esters.
- (4) Alkali salts of alkylaryl polyether sulfonates,
- (5) The alkanesulfonates.
- (6) Alkylphenyl polyethylene glycol ethers.
- (7) Alkali salts of fluoro-substituted alkanesulfonates.
- (8) Surfactants in which the hydrophilic fraction of the molecule is provided by ethylene oxide.
- (9) Alkyl phosphates.
- (10) Surfactant substituted amide reaction products of a carboxylic acid and ethanolamine.
- (11) Surfactant C<sub>8</sub> to C<sub>18</sub> alkyl chain esters of polyoxyethylene glycol.
- (12) Surfactant condensation products of a carboxylic acid and an amine.
- (13) Monoether surfactants.

In addition to the surfactant, phosphoric acid may be added to the composition of the instant invention to increase, to some degree, the adhesion of the coating composition to the metallic surface.

The composition of the instant invention is prepared by admixing the water-soluble chromium compound delineated above with the oxygenated organic compound also delineated above in the presence of water. While the exact reaction is unknown, it is thought that the oxygenated organic compound forms an oxidized complex and this results in an improved corrosion resistant coating.

In general in the compositions of the instant invention it is preferred to employ from about 0.05 to about 50 percent by weight of the oxygenated organic compound and from about 0.5 to about 10 percent by weight of the water-soluble of the chromium compound. As previously noted, phosphoric acid, in amounts from about 0.5 percent to about 10 percent have been found to be useful. With regard to the wetting agents or surfactants, if employed, amounts from about 0.01 percent to about 1 percent by weight are adequate. Preferably, the compositions of the instant invention include from about 0.5 to about 10 percent of the glycol ether and from about 2 to about 7 percent of the water-soluble chromium compound.

The instant invention will be illustrated by the following detailed examples. It is to be noted, however, that the instant invention is not deemed as being limited thereto.

## EXAMPLE 1

Coating formulations containing 20% glycol ether and 5.0% chromic acid were prepared by mixing equal volumes of the following two solutions.

Solution A: This solution, containing 40% glycol ether, was prepared by adding to a wide mouth jar.

|                                 | Grams |
|---------------------------------|-------|
| Ethylene glycol monobutyl ether | 40    |
| Water                           | 60    |

This mixture was shaken to dissolve at room temperature.

Solution B: A 10% solution of chromic acid in water was prepared by adding to a wide mouth jar.

|                   | Grams |
|-------------------|-------|
| Chromium trioxide | 10.0  |
| Water             | 90.0  |

This mixture was shaken to dissolve at room temperature.

Equal portions of Solutions A and B were mixed thoroughly at room temperature to give the desired coating formulation.

Coating formulations containing 12% glycol ether, 5.0% chromic acid and 0.5% phosphoric acid were prepared by mixing equal volumes of the following two solutions.

Solution C: This solution, containing 24% glycol ether, was prepared by adding to a wide mouth jar

|                                 | Grams |
|---------------------------------|-------|
| Ethylene glycol monobutyl ether | 24    |
| Water                           | 76    |

This mixture was shaken to dissolve at room temperature.

Solution D: This solution, containing 10.0% chromic acid and 1.0% phosphoric acid was prepared by adding to a wide mouth jar

|                     | Grams |
|---------------------|-------|
| Chromic trioxide    | 10.0  |
| 86% phosphoric acid | 1.0   |
| Water               | 89.0  |

This mixture was shaken to dissolve at room temperature.

Equal portions of Solutions C and D were mixed thoroughly at room temperature to give the desired coating formulation.

Solutions containing the other compositions listed in Table 1 were prepared in a similar fashion. The wetting agent, when used, was added by using the proper volume of a dilute (0.10%) aqueous solution of the wetting agent. Carbon steel (1010) panels were used for the rust inhibition test. These panels measured 3" x 8" x 0.051" and were cut from steel which had been cold rolled using rolls that yields a surface finish of 6-12 microinches. The panels had been protected from rusting with a vapor phase inhibitor and were used directly as received. The panels were dip-coated in the proper formulation, withdrawn from the solution and allowed to drain dry at room temperature. After standing at room temperature for 24 hours, the panels were placed in the QCT condensing humidity cabinet. The cabinet was operated with the water temperature at 131° F. and vapor temperature at 120° F. Rusting was induced by the moisture which condensed continuously on the panels. The panels were observed daily for the appearance of rust spots and were rated as follows. A perimeter approximately 1/4" wide was excluded from observation. A test surface passed if it contained no more than three dots of rust, no one of which was greater than 1 mm. in diameter. A test surface failed if it contained one or more dots of rust larger than 1 mm. in diameter or if it contained four or more dots of any size. The number of days protection obtained (days with no rust spots appearing) was a measure of product performance.

Table 1 shows the number of days of rust protection afforded to panels which had been coated with the rust inhibiting compositions described.

TABLE 1.—NUMBER OF DAYS OF RUST PROTECTION OBTAINED WITH COATINGS PREPARED WITH ETHYLENE GLYCOL MONO BUTYL ETHER CHROMIUM TRIOXIDE, PHOSPHORIC ACID OR WETTING AGENT AND WATER

| Test No. | Formulation composition, wt. percent |                   |                              |               |       | Days of protection from rust, QCT cabinet; panels air dried 24 hrs. at room temperature |
|----------|--------------------------------------|-------------------|------------------------------|---------------|-------|-----------------------------------------------------------------------------------------|
|          | Ethylene glycol mono butyl ether     | Chromium trioxide | Phosphoric acid <sup>1</sup> | Wetting agent | Water |                                                                                         |
| 1        | 20                                   |                   |                              |               | 80    | 0                                                                                       |
| 2        | 20                                   | 5                 |                              |               | 75    | 13                                                                                      |
| 3        | 50                                   | 5                 |                              |               | 45    | 16                                                                                      |
| 4        | 20                                   | 5                 | 1                            |               | 74    | 9                                                                                       |
| 5        | 12                                   | 5                 | 0.5                          |               | 82.5  | 16                                                                                      |
| 6        | 1                                    | 5                 | 0.5                          |               | 93.5  | 4                                                                                       |
| 7        | 1                                    | 5                 | 0.5                          | 2 0.5         | 91.45 | 28                                                                                      |
| 8        | 1                                    | 5                 | 0.5                          | 2 0.05        | 91.95 | 4                                                                                       |
| 9        | 0                                    | 5                 |                              |               | 95    | 1                                                                                       |
| 10       | 20                                   | 5                 |                              |               | 75    | 10                                                                                      |

<sup>1</sup> Commercial syrup phosphoric acid containing 85-87% H<sub>3</sub>PO<sub>4</sub>.

<sup>2</sup> Two ml. of a 0.1% aqueous solution of nonylphenoxypoly (ethyleneoxy) ethanol.

<sup>3</sup> Ethylene glycol monobutyl ether.

As will readily be seen from a study of the above table, the panels coated with ethylene glycol monobutyl ether and water, i.e., Test No. 1, showed evidence of rusting in less than 1 day and, in fact, in less than 1 hour. The panels coated with only chromic acid and water demonstrated rusting within 1 day. In contrast thereto, however, panels coated with the composition of the instant invention, i.e., a composition comprising a glycol ether, a chromium compound and water, were protected from rusting for a period of at least 4 days and in most instances for a substantially longer period.

placed, after various times of drying at room temperature or after oven curing from 10-15 minutes at 100° C., in the QCT cabinet for determination of rust protection. Table 2 shows the number of days rust protection obtained with these coatings prepared with the mono methyl and ethyl ethers of ethylene glycol, the mono methyl, ethyl and butyl ethers of diethylene glycol, and the mono propyl together with chromium trioxide, and phosphoric acid or wetting agent.

Five to greater than 10 days rust protection was obtained with all of these products.

TABLE 2.—NUMBER OF DAYS OF RUST PROTECTION IN THE QCT CABINET OBTAINED WITH COATINGS PREPARED WITH DIFFERENT GLYCOL ETHERS, CHROMIUM TRIOXIDE, PHOSPHORIC ACID OR A WETTING AGENT AND WATER

| Glycol ether, concentration            | Percent compositions of coating formulation |                            |                 |       | Air dried panels | Oven dried panels 10-15 min. at 100° C. |
|----------------------------------------|---------------------------------------------|----------------------------|-----------------|-------|------------------|-----------------------------------------|
|                                        | Chromium trioxide                           | Wetting agent <sup>1</sup> | Phosphoric acid | Water |                  |                                         |
| 5% ethylene glycol mono methyl ether   | 5                                           | 1                          |                 | 89    | 98               | >10                                     |
| 5% ethylene glycol mono ethyl ether    | 5                                           | 1                          |                 | 89    | 96               | >10                                     |
| 5% diethylene glycol mono methyl ether | 5                                           | 1                          |                 | 89    | 120              | >10                                     |
| 5% diethylene glycol mono ethyl ether  | 5                                           | 1                          |                 | 89    | 120              | >10                                     |
| 5% diethylene glycol mono butyl ether  | 5                                           | 1                          |                 | 89    | 120              | >10                                     |
| 5% propylene glycol mono propyl ether  | 5                                           |                            | 1               | 89    | 120              | 6                                       |
| 20% propylene glycol mono propyl ether | 5                                           |                            | 1               | 74    | 120              | 5                                       |

<sup>1</sup> Nonylphenoxypoly (ethyleneoxy) ethanol containing 64% ethylene oxide.

#### EXAMPLE 2

Coating formulations containing 50% glycol ether and 5.0% chromic trioxide were prepared by adding to a wide mouth jar

Ethylene glycol monobutyl ether \_\_\_\_\_ 50 Grams  
Water \_\_\_\_\_ 45

45

#### EXAMPLE 4

Aqueous coating solutions were prepared using chromium trioxide and the tri- and tetraethylene glycols listed in Table 3. Panels were air dried for 24, 120, or 168 hours and were oven cured for 15 min. at 100° C. The days rust protection obtained are listed in Table 3.

TABLE 3.—NUMBER OF DAYS RUST PROTECTION IN QCT CABINET OBTAINED WITH COATINGS PREPARED WITH TRI- AND TETRAETHYLENE GLYCOL ETHERS

|                                        | Percent composition of coating formulation |               |       | Days of protection from rust, QCT cabinet |              |                      |
|----------------------------------------|--------------------------------------------|---------------|-------|-------------------------------------------|--------------|----------------------|
|                                        | Chromium trioxide                          | Wetting agent | Water | Air dried panels                          | Hours drying | Days rust protection |
| 5% triethylene glycol dimethyl ether   | 5                                          | 1             | 89    | 120                                       | >10          | >10                  |
| 5% tetraethylene glycol dimethyl ether | 5                                          | 1             | 89    | 120                                       | >10          | >10                  |
| 5% triethylene glycol monomethyl ether | 5                                          | 1             | 89    | 120                                       | >10          | >10                  |
| 5% triethylene glycol mono ethyl ether | 5                                          | 1             | 89    | 120                                       | >10          | >10                  |
| 5% triethylene glycol mono butyl ether | 5                                          | 1             | 89    | 168                                       | >10          | >10                  |

This mixture was shaken to dissolve at room temperature. After solution had been obtained 5.0 grams of chromium trioxide was added.

The mixture was shaken at room temperature to dissolve.

Panels were then coated, dried at room temperature for 24 hours and tested as described in Example 1. Rust protection of 13 days was obtained.

#### EXAMPLE 3

Coating solutions having the compositions listed in Table 2 were prepared as described in Example 1 and

65  
Panels were coated with formulations having the compositions listed in Table 4, and were dried as described in the table headings. After drying, they were subject to impact using a four-pound hammer dropped from a height required to give 70 or 80 inch-pounds impact. The hammer had a hemispherical head which was 1/2" in diameter. These panels were then placed in the QCT cabinet to determine rust protection on the stressed surface. Observations were also made on the plane panel surface. The days protection obtained are listed in Table 3.

Examination of the data shows that excellent rust protection was obtained on the impacted surface.

What is claimed is:

1. A corrosion-resistant coating composition consisting

TABLE 4.—NUMBER OF DAYS RUST PROTECTION IN QCT CABINET AT 120° F. VAPOR TEMPERATURE

| Formulation ref. | Monobutyl-ether of ethylene glycol, percent | Percent CrO <sub>3</sub> | Percent H <sub>3</sub> PO <sub>4</sub> | Ethoxy-alkyl-phenol <sup>1</sup> | Percent water | Days rust protection |           |            |           |                    |                             |
|------------------|---------------------------------------------|--------------------------|----------------------------------------|----------------------------------|---------------|----------------------|-----------|------------|-----------|--------------------|-----------------------------|
|                  |                                             |                          |                                        |                                  |               | Impacted Area        |           | Plane area |           | Air dried 120 hrs. | Oven dried 100° C., 15 min. |
|                  |                                             |                          |                                        |                                  |               | 70 in.-lb            | 80 in.-lb | 70 in.-lb  | 80 in.-lb |                    |                             |
| 1                | 1.0                                         | 5.0                      | 0.5                                    | 0.05                             | 93.45         | >10                  | >10       | >3         | 3         | 7                  | 3                           |
| 2                | 1.0                                         | 5.0                      | 0.5                                    | 0.05                             | 93.95         | >10                  | >10       | 6          | 6         | 9                  | 6                           |
| 3                | 1.0                                         | 5.0                      | 0.5                                    | 0.05                             | 93.45         | 6                    | 8         | 7          | 14        | 6                  | 15                          |
| 4                | 2.0                                         | 5.0                      | 0.5                                    | 0.05                             | 93.45         | >16                  | 15        | >25        | >25       | 10                 | >25                         |
| 5                | 4.0                                         | 5.0                      | 0.5                                    | 0.05                             | 93.45         | >11                  | 3         | 11         | 8         | 11                 | 12                          |
| 6                | 6.0                                         | 5.0                      | 0.5                                    | 0.05                             | 93.45         | 8                    | >21       | >21        | 20        | >21                | 20                          |

<sup>1</sup> C<sub>12</sub>-18 alcohol plus 70% ethyleneoxide.

<sup>2</sup> Nonylphenoxy poly (ethyleneoxy) ethanol containing 64% ethylene oxide.

### EXAMPLE 6

Coating formulations containing 5.0% chromium trioxide and 1% H<sub>3</sub>PO<sub>4</sub>, with 5.0% of either triethylene glycol monomethyl ether, triethylene glycol monoethyl ether, or triethyleneglycol monobutylether, were prepared as in Example 1. Steel panels were coated, air dried for 48-120 hours and placed on the QCT cabinet for evaluation of rust protection. These formulations gave poor coatings and rust inhibition. However, when 1.0% wetting agent was added to the formulation, instead of 1% H<sub>3</sub>PO<sub>4</sub>, excellent coatings were produced and rust protection extending to greater than 21 days was obtained. This is shown in Table 5.

TABLE 5.—RUST PROTECTION BY ETHERS OF TRIETHYLENE GLYCOL, COATING COMPOSITION, PERCENT

All formulations contained 5.0% glycol ether, 5.0% CrO<sub>3</sub>, and 89.0% water

| Glycol ether<br>RO(C <sub>2</sub> H <sub>4</sub> O) <sub>3</sub> H | H <sub>3</sub> PO <sub>4</sub> | Wetting agent <sup>1</sup> | Days rust protection in QCT cabinet |                             |                             |
|--------------------------------------------------------------------|--------------------------------|----------------------------|-------------------------------------|-----------------------------|-----------------------------|
|                                                                    |                                |                            | Air dried 48-120 hrs.               | Oven dried 15 min., 100° C. | Oven dried 100° C., 15 min. |
| R=Methyl                                                           | 0.0                            | 1.0                        | >21                                 | >21                         | >21                         |
| R=ethyl                                                            | 0.0                            | 1.0                        | >21                                 | >21                         | >21                         |
| R=butyl                                                            | 0.0                            | 1.0                        | >21                                 | >21                         | >21                         |

<sup>1</sup> Nonylphenoxy poly (ethyleneoxy) ethanol containing 64% ethylene oxide.

As will readily be seen from a study of Table 5, the compositions of the instant invention, including phosphoric acid and a wetting agent, provided superior rust protection.

### EXAMPLE 7

Coating formulations were prepared as in Example 1 containing 5.0% and 20.0% of the dimethyl ethers of tri- and tetraethylene glycol with 5.0% chromic acid. Some of the solutions contained phosphoric acid; some of them contained a wetting agent. The composition and performance data are shown in Table 6. Some panels were air dried for 24-120 hours; some were oven dried for 15 min. at 100° C.

TABLE 6.—RUST PROTECTION BY DIMETHYL ETHERS OF TRI- AND TETRAETHYLENE GLYCOL COATING COMPOSITION, PERCENT

All formulations contained 5.0% CrO<sub>3</sub> and sufficient water to make 100.00%

| Dimethyl glycol ether of tri-, tetra-ethylene glycol | H <sub>3</sub> PO <sub>4</sub> | Wetting agent | Days rust protection in QCT cabinet |                             |                             |
|------------------------------------------------------|--------------------------------|---------------|-------------------------------------|-----------------------------|-----------------------------|
|                                                      |                                |               | Air dried 48-120 hrs.               | Oven dried 15 min., 100° C. | Oven dried 100° C., 15 min. |
| 5.0% triethylene glycol                              | 1.0                            | 0.0           | 2                                   | 2                           |                             |
| 20.0% triethylene glycol                             | 1.0                            | 0.0           | 1                                   | 1                           |                             |
| 5.0% triethylene glycol                              | 0.0                            | 1.0           | 5                                   | 10                          |                             |
| 5.0% tetraethylene glycol                            | 1.0                            | 0.0           | 1                                   | 1                           |                             |
| 20.0% tetraethylene glycol                           | 1.0                            | 0.0           | 1                                   | 1                           |                             |
| 5.0% tetraethylene glycol                            | 0.0                            | 1.0           | 28                                  | 17                          |                             |

<sup>1</sup> Nonylphenoxy poly (ethyleneoxy) ethanol containing 64% ethylene oxide.

Once again, it will readily be noted that the compositions of the instant invention provide a surprising and unexpected rust protection for metallic surfaces.

75

11. The composition of claim 5 wherein the compound having the structure of Formula I is the monoalkyl ether of triethylene glycol.

essentially of the product of the reaction in the presence

20 of water, of a water-soluble chromium compound and a compound having the formula:



25 wherein R<sub>1</sub> is an alkyl group having from 1 to 6 carbon atoms, R<sub>2</sub> and R<sub>3</sub> are selected from the group consisting of hydrogen and an alkyl group having from 1 to 6 carbon atoms, and n is an integer of from 1 to 4; said chromium compound being present in an amount of from about 0.5 to about 10% by weight and said compound of Formula I being present in an amount of from about 0.5 to about 50% by weight.

2. The composition of claim 1 wherein said chromium compound is present in an amount of from about 2 to about 7% by weight.

3. The composition of claim 1 wherein said compound of Formula I is present in an amount of from 0.5 to about 10% by weight.

4. The composition of claim 1 in the form of an aqueous solution thereof.

5. A corrosion-resistant coating composition according to claim 1 additionally including at least one member selected from the group consisting of phosphoric acid, and compatible anionic and non-ionic surfactants.

6. The composition of claim 5 wherein the water-soluble chromium compound is chromium trioxide.

7. The composition of claim 5 wherein the compound having the structure of Formula I is the monobutyl ether of ethylene glycol.

8. The composition of claim 5 wherein the compound of Formula I is the monoalkyl ether of ethylene glycol.

9. The composition of claim 5 wherein the compound having the structure of Formula I is the monoalkyl ether of diethylene glycol.

10. The composition of claim 5 wherein the compound having the structure of Formula I is the monoalkyl ether of propylene glycol.

12. The composition of claim 5 wherein the phosphoric acid is present in an amount of from about .05 to about 10 percent.

13. The composition of claim 5 wherein the surfactant is present in an amount of from about 0.01 to about 1 percent.

14. The composition of claim 5 wherein the compound having the structure of Formula I is monobutyl ether of ethylene glycol.

15. A process for improving the corrosion resistance 10 of metallic surfaces which comprise contacting a metallic surface with a composition according to claim 1 whereby there is formed a corrosion-resistant film upon said surface and allowing said film to dry thereon.

16. The process of claim 15 wherein said composition 15 is in the form of an aqueous solution thereof.

17. A process for improving the corrosion resistance of metallic surfaces according to claim 15 wherein said composition additionally contains at least one member selected from the group consisting of phosphoric acid and 20 anionic and non-ionic surfactants.

18. The process of claim 15 wherein the chromium compound is chromium trioxide.

19. The process according to claim 15 wherein the drying is effected at temperatures in the range from room 25 temperature up to 100° C.

20. The process of claim 17 wherein the phosphoric acid is present in an amount of from about .05 to about 10 percent.

21. The process of claim 17 wherein the surfactant is present in an amount of from about 0.01 to about 1 percent.

#### References Cited

##### UNITED STATES PATENTS

|           |         |               |       |          |
|-----------|---------|---------------|-------|----------|
| 2,662,835 | 12/1953 | Reid          | ----- | 252—396  |
| 3,189,489 | 6/1965  | Schiffman     | ----- | 148—6.16 |
| 3,218,265 | 11/1965 | Rink et al.   | ----- | 252—389  |
| 3,279,958 | 10/1966 | Maurer et al. | ----- | 148—6.16 |
| 3,445,400 | 5/1969  | Everhart      | ----- | 21—2.7   |

##### FOREIGN PATENTS

|         |         |               |       |         |
|---------|---------|---------------|-------|---------|
| 683,154 | 11/1952 | Great Britain | ----- | 252—389 |
|---------|---------|---------------|-------|---------|

LEON D. ROSDOL, Primary Examiner

I. GLUCK, Assistant Examiner

##### U.S. CL. X.R.

21—2.7; 106—14; 148—6.2; 252—389; 260—438.5 R